

# UNITED STATES PATENT OFFICE.

JAMES ALVAH BLANCHARD, OF BROOKLYN, NEW YORK.

## COMPOSITION FOR LINING VESSELS.

SPECIFICATION forming part of Letters Patent No. 380,853, dated April 10, 1888.

Application filed June 3, 1887. Serial No. 240,187. (Specimens.)

*To all whom it may concern:*

Be it known that I, JAMES ALVAH BLANCHARD, of the city of Brooklyn, in the county of Kings and State of New York, have invented 5 a new and useful Composition of Matter, of which the following is a full, clear, and exact description.

My invention relates to a composition of matter for coating the interior of boxes, wraps, or other casings and packages to fit them for use in inclosing compounds of a corrosive 10 nature, either in a solid, fluid, or semi-fluid state; and its objects are to preserve the quality of the inclosed compound, to prevent 15 access of air thereto and emanations of noxious gases therefrom, and also to prevent the inclosed compound from corroding and destroying the wrapper or casing, and thus exposing and injuring or destroying adjacent and 20 surrounding objects.

Chloride of lime is such a compound as I have above mentioned, and is an article in general use throughout the country for deodorizing, disinfecting, and bleaching purposes. When exposed to the air, it evolves 25 chlorine gas, which has a peculiarly pungent and disagreeable odor and is deleterious to health, and also has the effect of tarnishing metal articles which are exposed to its influence. Chloride of lime when so exposed to 30 the air also absorbs moisture therefrom and becomes actively corrosive in its nature and destroys whatever envelops it, as well as whatever else it comes in contact with in its exit 35 from its casing. For the reasons above stated its purchase and sale in either large or small quantities is undesirable, unless it is inclosed in wrappers or casings which will resist corrosion and prevent ingress of air or egress of 40 gases to and from it. With a view to obviate these objections, metallic sheets and tin-foil have been made use of to inclose this chloride; but such is its corrosive action and so rapidly 45 does it take place that, aided by the porosity of the inclosing material, holes are soon eaten in the box or package, the compound exudes therefrom, giving forth its noxious gas, injuring and destroying its surroundings, and when 50 it is exposed to the air becoming useless for commercial purposes.

Boxes or packages constructed of wood or

materials of vegetable and animal origin—such as cloth of various kinds, paper, pasteboard, canvas, parchment, &c.—are equally unavailable of themselves for inclosing such a 55 compound, inasmuch as their porosity permits air to have access to their contents, allows the gas to escape therefrom, they are not proof against the corrosive action of their contents, and the compound has the same effects 60 upon its surroundings as when inclosed in metallic sheets or tin-foil.

The object of my invention is to provide a comparatively inexpensive composition of matter the ingredients of which may be readily 65 assimilated, and which may be quickly applied to the material constituting the box or package before or after the same is given proper shape, and thus preclude the entrance of air to the contained compound, the escape of gas 70 therefrom, destruction or injury to the inclosing material, or exit of the compound itself, whereby compounds having the characteristics I have mentioned may be exposed for sale or kept in reserve without the attendant 75 disagreeable features to which allusion has been made.

My composition of matter consists of the following-named ingredients, combined in substantially the proportions stated, namely: 80 resin, eighty pounds; black pitch, sixty pounds; gypsum, forty pounds; petrolatum, twenty-five pounds, and combined in the following manner:

I first expose the resin and black pitch to 85 heat in a kettle or other suitable receptacle, stirring them briskly as they melt, and when they have become liquefied and well mixed together I stir in the gypsum. When the three ingredients have become thoroughly 90 mixed, I add the petrolatum and stir the whole mass until all its components are completely assimilated. As the gypsum has a tendency to fall to the bottom of the receptacle when the liquid is at rest, the composition should 95 be well stirred before applying it to use. The composition of matter thus produced is comparatively inexpensive, and by virtue of the nature and attributes of its ingredients and the manner in which they are assimilated, as 100 herein described, when applied to the box or package, renders the same air-tight and proof

against the corrosive and disintegrative action of its contents, and also enables the package to withstand any degree of cold and any degree of heat up to 120° Fahrenheit, applied externally. These properties of my invention allow of the employment in the construction of the receptacle of any of the hitherto ineffective materials and permit the casing to be used for inclosing compounds, either in a solid, fluid, or semi-fluid state, of a disintegrative and corrosive nature, protecting them from the action of heat, cold, or air, and preventing their escape in a gaseous, solid, or fluid form.

15 The form of the receptacle, the material to be used in its construction, and the means and manner of fastening it after it is filled may be in each particular such as is deemed suitable

and preferable to the manufacturer and packer, and my composition of matter may be applied to it in any suitable manner. 20

What I claim, and desire to secure by Letters Patent of the United States, is—

As a new article of manufacture, the herein-described composition of matter for rendering 25 air-tight and proof against corrosion wrappers or casings for holding chloride of lime and like corrosive compounds, consisting of resin, black pitch, gypsum, and petrolatum, combined in substantially the proportions 30 herein specified.

JAMES ALVAH BLANCHARD.

Witnesses:

F. W. HANAFORD,  
C. SEDGWICK.